

Aug. 8, 1950

R. A. CARLETON

2,517,838

## DRYING OIL

Filed March 2, 1943

5 Sheets-Sheet 1

Fig. 1a.



## INVENTOR

Robert A. Carlton  
by William D. Wharton  
his attorney

Aug. 8, 1950

R. A. CARLETON

2,517,838

## DRYING OIL

Filed March 2, 1943

5 Sheets-Sheet 2



## INVENTOR

Robert A. Carleton  
by William T. Wharton  
his attorney

Aug. 8, 1950

R. A. CARLETON

2,517,838

DRYING OIL

Filed March 2, 1943

5 Sheets-Sheet 3

*Fig. II.*



*Fig. III.*



INVENTOR

Robert A. Carleton  
by William B. Wharton  
his attorney

Aug. 8, 1950

R. A. CARLETON

2,517,838

DRYING OIL

Filed March 2, 1943

5 Sheets-Sheet 4

Fig. IV.



Fig. V.



Fig. VI.



Robert A. Carlton  
by William D. Wharton  
his attorney

Aug. 8, 1950

R. A. CARLETON

2,517,838

DRYING OIL

Filed March 2, 1943

5 Sheets-Sheet 5

*Fig. VII.*



INVENTOR

Robert A. Carleton  
by William T. Wharton  
his attorney

## UNITED STATES PATENT OFFICE

2,517,838

## DRYING OIL

Robert A. Carleton, Mamaroneck, N. Y.

Application March 2, 1943, Serial No. 477,723

5 Claims. (Cl. 260—405.5)

2

**1** This invention relates to a method of producing drying oils of improved drying and film-forming properties, from drying oils of non-conjugate type.

My invention primarily relates to a treatment of non-conjugate type glyceride oils containing large amounts of glycerides having 18 or more atoms in the carbon chain, at least two pairs of which are united by double bonds, by which treatment new double bonds are introduced and rearrangement of double bonds in the carbon chain to give a conjugate rather than a non-conjugate structure is effected. It is to be understood further that my invention involves the introduction of double bonds into determinate positions in the carbon chain of the oil molecules; and that it involves both an increase in the total number of double bonds linking particular unsatrate carbon atoms of the carbon chain, and in such positioning of these carbon atoms in the carbon chain that approximately all the introduced double bonds are in conjugate relation.

My invention concerns itself with the well-known fact that in drying oils, the rapidity with which they dry and the hardness of the film which they produce is affected not only by the total unsaturation of the oil, or number of double carbon bonds which it contains; but that those desirable properties of the drying oil are affected greatly by the arrangement of the unsaturated linkages, or double carbon bonds, in the oil molecule. It is well understood that each drying oil is composed of a varying number of components, which in instances present great differences in the order of their unsaturation, and in the arrangement of their double carbon bonds. The above is to be taken generally as referring to each commercial drying or semi-drying oil, such as linseed oil, soya bean oil, etc., and in its relation specifically to the order of unsaturation and the order of conjugation is to be taken also as relating to the individual components of the oils, such as the glycerides of linoleic acid, and the glycerides of linolenic acid.

My invention concerns itself also with a finished drying oil product which by virtue of the total treatment to which it has been subjected is composed in substantial entirety of desired components useful in the composition of the oil. In both connections it concerns itself with the order of hydroxylation and condensive dehydrogenation which is effected; and with the conduct of such treatments in a manner which leads wholly to improvement in the properties of the drying oil product which is recovered, and in a manner to obtain

in determinate order the physical and chemical changes giving the desired product.

As is well-known, China-wood oil may be taken as exemplifying drying oils having most of their double bonds in conjugate relation, another and less known member of the class being oiticica oil. While the total unsaturation of China-wood oil, as represented by its iodine absorption index, is substantially less than the total unsaturation of linseed oil or perilla oil, China-wood oil dries much more rapidly than do those other and non-conjugate oils, and has the ability to form films which have a hardness and a resistance to water and chemicals substantially greater than that of the more unsaturated oils, the unsaturated glycerides of which present as an average no substantial conjugation. Thus, China-wood oil is composed largely of the highly reactive glyceride of eleostearic acid, in which substantially all the double bonds present are in conjugate relation. As is well-known, that oil polymerizes or gels at equal temperatures many times faster than the more unsaturated but non-conjugate and relatively less reactive linseed oil. As noted, there is substantial difference in the type of film formed by conjugate type oils and the non-conjugate type oils; because the conjugate oils form films which are characterized by "through drying" to give hard and highly resistant coatings, whereas the films of non-conjugate oils dry from the surface, so that the underlying regions of the film dry slowly, and the film does not have the hardness and resistance of a film composed of the conjugate type oils.

35. It is generally considered that the non-conjugate type glyceride oils owe their drying properties chiefly to their inclusion of unsaturated linoleic acid glycerides having two double carbon bonds in the 9-10 and 12-13 positions and an iodine value of about 181, and to linolenic acid glycerides having three double carbon bonds in the 9-10, 12-13, and 15-16 positions, and an iodine value of about 274. In addition the oils contain glycerides of oleic acid and of saturate acids, having little or no drying power. The glyceride of oleic acid has one double carbon bond in the 9-10 position, and has an iodine value of about 89. In addition to a substantial content of linoleic, linolenic, and oleic acid glycerides, fish oils having drying properties, such as sardine oil and menhaden oil, contain substantial amounts of other unsaturated non-conjugate fatty acid glycerides having from 4 to 6 double bonds in the carbon chain.

As has been above indicated, the proportions of the several saturate and unsaturate fatty acid glycerides occur in the various oils in greatly varied proportions, to form mixed triglycerides. Certain oils, such as cotton seed oil and corn oil, while containing substantial amounts of linoleic acid glycerides, also contain a large proportion of saturate fatty acid glycerides and of oleic acid glyceride. These oils, of which I may take cotton seed oil and corn oil as exemplary, are not, therefore, commonly considered to be drying oils. These examples of such oils as have iodine values over 100, may be used alone or in mixtures as the starting oil for my process.

My present invention involves the discovery that by hydroxylating and then condensively dehydroxylating unsaturate non-conjugate glycerides of fatty acids there are introduced in the carbon chains of the oil molecules an increased number of double carbon bonds in determinate positions and in conjugate relation. I have discovered that this hydroxylation and attendant condensive dehydroxylating, with introduction of double carbon bonds in determinate conjugate relation may be effected selectively to impart to the oil increased tendency readily to polymerize which is of measured order.

Concretely I have discovered that the reactivity of fatty acid glycerides having 18 or more carbon atoms and two or more double bond linkages in the carbon chain may be greatly increased by hydroxylating followed by condensive dehydroxylating to introduce new double carbon bonds and to increase conjugation in the carbon chains of the oil molecules, and that the hydroxylating and consequently the dehydroxylating may be selective as to the number and positions of the unsaturate carbon atoms which are involved. This involves the further discovery that the determinate positions in which dehydroxylating based upon precedent hydroxylating is effected in drying oils of that type are such as to give maximum effectiveness in increased reactivity to the increased unsaturation and the conjugation which has been introduced.

The hydroxyl group addition to the unsaturate carbon atoms, which comprises the first step in my novel process, is effected by reaction of the oil with oxygen in the presence of water, and any suitable and convenient reagents and procedure for so doing may be employed.

In exploring the mechanism, I have found that epoxide formation and hydroxyl addition to the unsaturate carbon atoms in the glyceride molecules may be accomplished in various ways. One manner of accomplishing this is to treat the starting oil with air or other oxygen-containing gas, with or without the use of oxidation catalysts, and effecting the hydroxylating predicated upon epoxide formation by conducting the oxidation procedure in the presence of steam or water, so that epoxide formation is accompanied immediately by hydration. Another procedure by which hydroxyl addition is accomplished is by treating the oil with water solutions of compounds which readily give up oxygen, such for example as potassium permanganate or hydrogen peroxide. A still further example of procedure for effecting hydroxyl addition at unsaturate carbon atoms of the glycerides is to effect epoxide formation immediately resulting in hydroxylating, by reacting and decomposing a water solution of oxygen-containing compounds such as sodium carbonate with a reagent therefor such as gaseous chlorine, with subsequent liberation of

free oxygen, which reacts with the unsaturate carbon atoms present to add hydroxyl groups thereto. It is possible also to combine these procedures as by treating the oil with air and with a water solution of an oxygenating compounds, such as potassium permanganate.

The above recited procedures are to be taken as illustrative of treatment by which the fact of hydroxylating in the oil molecules may be attained, and not as limitations upon my invention. It is to be understood that hydroxylating of itself serves to decrease rather than to increase the unsaturation and reactivity of the oil. When, however, the hydroxylating is associated or combined with condensive dehydroxylating a marked increase in unsaturation and reactivity of the treated over the untreated oil is accomplished.

Dehydroxylating is effected by condensation between the added hydroxyl groups and hydrogen atoms of the original molecular structure under the influence of heat and preferably also with a condensive dehydroxylating catalyst and under substantially anhydrous conditions. Assuming that dehydroxylating is effectively performed, the increased unsaturation and the conjunction effected in the glycerides of the oils depends upon the order of hydroxylating which has been effected in them. Consequently, the order in which unsaturation is increased and conjugation created in the treated glycerides is controllable by selectivity in the precedent hydroxylating.

Selectivity in the treatment of the oil to increase its unsaturation and conjugation is an important consideration. If we consider linseed oil as the starting material for my treatment, it has been above noted that the composition of such oil is approximately 24% linolenic acid glyceride, 62% linoleic acid glyceride, 5% oleic acid glyceride, and 9% saturate acid glycerides. Linoleic acid has in its carbon chain two double carbon bonds in the 9-10 and 12-13 positions. If then we consider that the acid is completely hydroxylated to form tetrahydroxystearic acid and then is subjected to condensive dehydroxylating, four of the original atoms of hydrogen are removed from the molecule and four conjugated double carbon bonds are introduced in the 7-8, 9-10, 11-12, and 13-14 positions. Similarly linolenic acid has in its carbon chain double bonds in the 9-10, 12-13, and 15-16 positions. When there is complete hydroxyl group addition to form hexahydroxystearic acid, followed by condensive dehydroxylating, the result is to remove six of the original hydrogen atoms and to introduce double bonds in the 6-7, 8-9, 10-11, 12-13, 14-15, and 16-17 positions. Mechanism of a condensive dehydroxylating reaction is rather complex, and not completely understood. In view, however, of the results attained, it is quite probable that due to strains set up in the molecule by the relatively high reacting temperature and atomic recombinations, there is first a migration of the relatively mobile hydrogen atoms with resulting shift in position of the active carbon atoms, to permit condensation between the added hydroxyl group and an adjacent hydrogen atom to form the above indicated double bond arrangement, without substantial formation of objectionable ring compounds.

I have found that because of an inherent selectivity, or difference in the degree of reactivity toward epoxidation exhibited by the several unsaturate carbon atoms in the oil molecule, depending upon their relative position in the carbon chain, and by the quantitative and selective

regulation of the variables affecting the hydroxyl group addition to the unsaturated carbon atoms, the starting oil may be treated by the present invention to have a lesser or greater determinate degree of unsaturation and conjugation with consequent variation in its heat-reactivity within the aforesaid range. It may be here noted that the position of the unsaturate carbon atoms in the molecules of a drying oil has a great influence on the reactivity of the oil. Unsaturation, and more particularly conjugate unsaturation, tends more greatly to heat reactivity and oxygen-reactivity of the oil the closer it is to the glycerol radical of the oil molecule. It is an important aspect of my process, as will hereinafter appear more specifically, that in it unsaturation, and unsaturation in conjugate relation, is introduced directly and permanently in determinate positions and that such positions are favorable to high reactivity of the product oil.

The initial factor in my process is the ability of unsaturate carbon atoms to react additively with oxygen to form epoxide, which in the presence of water immediately hydrates to form a hydroxyl group addition. I have found further that when two or more pairs of such carbon atoms are present the position of the carbon atoms so linked in the carbon chain greatly influences their relative reactivity with oxygen. Thus if linoleic acid glyceride be considered, the carbon atoms in the 9-10 position require greater stimulus to cause their reaction with oxygen than is required by the carbon atoms in the 12-13 position. In linolenic acid glyceride the carbon atoms in the 15-16 position in like manner have greater reactivity than the carbon atoms in the 9-10 position, and they in turn have greater reactivity with oxygen than the carbon atoms in the 12-13 position.

The exercise of selectivity in the hydroxylation of the oil involves many variables which by usual and known procedure may be applied to each individual operation, the intent to effect selectivity being present and procedural guides of general sort being had. The quantity of oxygen which may be rendered available from the oxygen-supplying substance used in the process may be taken as the primary guide with respect to the desired theoretical epoxide formation and hydroxyl addition to the oil molecule. The supply of water and its contact with the oil involved in hydroxylation should be ample to effect substantially complete and immediate hydration of the epoxide addition. The efficiency of the procedure by which epoxide formation is effected may then be considered, and this involves as variables the activity of the oxygen-supplying reagent, the time-temperature and pressure factors, the quantity and effectiveness of the oxidation catalyst if such catalyst be used, and the effectiveness of contact between the oil molecules and the source of oxygen.

In all the important non-conjugate drying and semi-drying oils the preponderant fatty acid glycerides are the linoleic acid glyceride having 18 carbon atoms and two points of unsaturation in its carbon chain and linolenic acid glyceride having 18 carbon atoms and three points of unsaturation in its carbon chain. It may be stated broadly that the response of any starting oil, or mixture of starting oils, to my process corresponds closely to the quantity of unsaturates of that sort which it contains. In obtaining selectivity in the practice of my invention it is therefore a simple matter to adjust the variables in con-

formity with altered compositions of the starting oil.

In my process it is not necessary catalytically to stimulate the mechanism by which epoxidation occurs and the hydroxyl groups are added to the carbon atoms. When it is deemed expedient to accelerate the activity of the oxygen-supplying medium in effecting hydroxylation, epoxidation may be promoted by adding to the oil subjected to treatment a suitable quantity of well-known oxidation catalysts including the compounds of oxidizing metals used as dryers in coating compositions.

Good oil-oxygen contact is important from the view point of selectivity and from the view point of obtaining the desired order of treatment in the entire volume of oil treated. If high oil-oxygen contact efficiency is obtained, regulation of the other variables of the process to obtain approximate uniformity and selectivity in the changes appearing in the product oil is facilitated. Thus if the contact factor approaches maximum efficiency, the time of treatment is shortened, and the quantity of oxygen rendered available in reaction with the oil approaches closer to the quantity supplied by the oxygen-containing reagent in effecting the desired theoretical epoxide formation and hydroxylation.

It is convenient during the hydroxylation stage of the process to check the progress or extent of hydroxylation of the oil undergoing treatment, and such checking is facilitated in a continuous operation in which fully treated samples repeatedly may be taken, in which there is substantial uniformity throughout the body of the oil being treated, and in which the variables are particularly well under control. Thus the decrease in unsaturation caused by the hydroxylation may be determined by well-known and usual tests for change in iodine and hydroxyl value. By observing the results of such tests appropriate changes in the variables involved in the hydroxylation procedure may be made to deliver for condensive dehydroxylation oil which has been hydroxylated to the extent desired.

The subsequent step of condensive dehydrogenation, which as is well-known involves the removal of a hydrogen atom from the oil molecule to combine with a hydroxyl group to form water, is effected primarily by heat. This is illustrated by prior practice in the "dehydration" of castor oil in which one hydroxyl group initially is present.

The time-temperature variable in the condensive dehydroxylation quite commonly is decreased by the use of a dehydrating catalyst. A typical activating dehydration treatment for castor oil is to hold the oil at a temperature of about 400° F. to 500° F. for 2 to 3 hours, using a substantial quantity up to .4% or .5% the weight of the oil of a suitable dehydrating catalyst, such as the salt of a non-oxidizing acid. "Dehydrated" castor oil is, however, much less heat-reactive than my product oils. Thus China-wood oil under standard gelatin test condition usually polymerizes to a substantially dry gel in 10 to 12 minutes at a temperature of 540° F. At that temperature the usual "dehydrated" castor oil requires 40 or more minutes to polymerize to a gel, and untreated linseed oil requires from 280 to 300 minutes to polymerize to a sticky gel. In my process linseed oil hydroxylated moderately as above described polymerizes upon condensive dehydroxylation to a substantially dry gel in 10 to 12 minutes at a temperature of 540° F., and polymerizes to a sub-

stantially dry gel in 3 to 5 minutes at a temperature of 600° F.

The condensive dehydroxylation stage of my process thus presents a problem which is not met in the treatment of castor oil. Because of the high heat reactivity of the oil which is subjected successively to hydroxylation and to condensive dehydroxylation in accordance with my invention, there is a tendency for the oil strongly to polymerize immediately upon dehydration. If then this stage of the process be carried on in a relatively large mass of the oil, the dehydrated oil tends rapidly to polymerize and to pass to a stage of high viscosity or gelation before it can be cooled below its polymerization temperature.

I employ a "flash" dehydration procedure, by which the hydroxylated oil is condensively dehydrated with relatively slight increase in its viscosity. Desirably such "flash" dehydration is so conducted that water from the reaction is removed from the oil substantially as it is formed, and it depends primarily upon raising the oil very rapidly, in substantially less than one minute, to a temperature much higher than commonly employed in dehydrating castor oil, for example, a temperature of from about 500° F. to 700° F. and even higher, and upon substantial completion of the reaction immediately cooling the oil below its active polymerization temperature. In such procedure the oil is so presented for heating, as in a thin film, that its heat-absorption is very rapid and the oil moves rapidly through the zone in which it is treated.

Exemplary apparatus in which the method of my invention in its variant embodiments may be practiced is shown in the accompanying drawings, it being understood that the apparatus herein shown is illustrative only of many forms and types of apparatus which conceivably may be employed while conforming to the method of my invention.

In the drawings:

Fig. Ia is a diagrammatic view showing one form of apparatus for practicing the hydroxylation step or stage of my method.

Fig. Ib is a diagrammatic view showing associated apparatus for conducting the dehydroxylation step or stage of my method.

Fig. II is a cross-sectional view through the hydroxylation reactor shown in Fig. Ia taken in the plane of the section line II—II of Fig. Ia, and showing in detail one of the elements of the said hydroxylation reactor which are organized to provide contact between the oil subjected to treatment and the reagent, or reagents, with which it is treated.

Fig. III is a vertical sectional view through the contact element of Fig. II taken in the plane of the section line III—III of Fig. II.

Fig. IV is a fragmentary vertical sectional detail view taken through the upper region of the dehydration reactor shown in Fig. Ib, the portion of the reactor shown being embraced by the bracket line IV—IV of Fig. Ib.

Fig. V is a fragmentary vertical sectional detail view taken through the dehydration reactor of Fig. Ib in a region intermediate the height of the reactor, and embraced by the bracket line V—V of Fig. Ib.

Fig. VI is a fragmentary vertical sectional detail view taken through the lower region of the dehydration reactor shown in Fig. Ib, embraced by the bracket line VI—VI of Fig. Ib, and showing connections to the lower region of the dehydration reactor.

Fig. VII is a diagrammatic view of modified

hydroxylation apparatus, which may be utilized in place of the apparatus shown in Fig. Ia in operative association with suitable dehydrogenation apparatus, such suitable dehydrogenation apparatus being exemplified by that shown in Fig. Ib of the drawings.

Referring initially to Fig. Ia and to Figs. II and III of the drawings, reference numeral 1 designates an oil feed pump which, by way of inlet connection 2 supplies oil for treatment to hydroxylating reactor 3. A pump 4 supplies water, which may be if desired a reactive water solution, and which preferably is mildly alkaline, to the reactor 3 by way of an inlet 5.

Primarily considered, reactor 3 is a cylindrical columnar vessel which preferably is constructed of metal resistant to the corrosive action of the materials contained by it during the progress of the reaction, and is of suitable cross-sectional area and height to maintain continuously flowing streams of oil undergoing treatment and treating reagents for the oil at suitable reaction temperatures, for suitable periods of time to effect the desired hydroxylation of the oil. Reactor 3 is provided with a plurality of contact, or reaction, trays 6 arranged at spaced intervals throughout its height and purposed to effect intimate contact between the oil subjected to treatment and the reagent, or reagents, with which it is treated.

Reaction trays 6, as is shown in detail in Figs. II and III of the drawings, comprise each an upper plate 7 and a lower plate 8, spaced apart to form a temperature controlling jacket space 9, provided with inlet connections 10 and outlet connections 11, for the supply of heating and cooling medium, and with circulation-directing baffles 12. A plurality of bubble caps 13, which are preferably as shown of rectangular type, and which have closely spaced narrow slots 14 adjacent their lower edges, are supported a suitable distance above plate 7 and enclose the discharge ends of vapor ducts 15, the lower portions of which pass in vapor-tight manner through jacket spaces 9, and which have their upper openings 16 in discharge relation with the upper regions of the chambers within the bubble caps 13. Interconnection, or down, pipes 17 provide for the flow of liquid from the trays 6 to successive lower trays of the system. These down pipes 17 have their upper intake ends 18 outside the bubble caps of the several trays with which they are associated, and positioned a suitable height above the plate 7 of each of the trays, to maintain a determinate depth of the liquid flowing over the trays. The lower outlet ends 19 of the down pipes 17 are sealed against vapor flow by submergence an adequate distance in the liquid of the tray 6 lying next below the tray from which they provide overflow connection.

Speaking in terms of my method, continuously flowing streams of oil subjected to treatment and oxidizing and hydrating reagents introduced respectively by way of inlets 2 and 5 are supplied to the uppermost of the reaction trays 6 by supply connections 20 and 21, which discharge immediately above the upper surface 7 of the uppermost trays 6, at the space 22 outside bubble caps 13.

This oil surrounds and moves between bubble caps 13 in a sinuous manner, being drawn off by way of down pipe 17 at a level which is a suitable height, such as about 1½", above plate 7. In accordance with usual procedure, the inlet 18 of down pipe 17 is remote from the openings of

supply connections 20 and 21, thus to cause movement of the oil past the several bubble caps 13 of the tray. In each of the underlying trays, the discharge end of down pipe 17 leading from the tray next above takes the place of supply connections 20 and 21, but otherwise the arrangement is identical.

The oil subjected to treatment thus passes progressively downward through the reactor, and in its passage encounters an upwardly rising gaseous oxygen-containing medium, preferably air, which is pre-heated to a suitable determinate hydroxylating reaction temperature, such as a temperature from about 130° F. to 250° F., and which is supplied at a rate suitable for effecting hydroxylation in desired order.

Such gaseous oxygen-containing medium, which will be hereinafter spoken of illustratively as "air," enters space 24 in reactor 3, at inlet 23, and passes by way of vapor ducts 15 into bubble caps 13, from which it issues into the surrounding oil on the several plates 7, in the form of finely-divided bubbles, by way of slots 14 in the bubble caps. The air thus intimately contacts and agitates the stream of oil passing over the several reaction trays 6, and intimately mixes with the oil in reactive contact therewith. The residual air separating from the oil in the uppermost reaction tray 6 passes from the reactor by way of vapor discharge connection 25.

The air thus brought into contact with the oil streams passing over trays 6 serves the dual purpose of agitating the oil and mixing it with any oxidizing agent, additional to the air, which may be used in this step of the process, and also supplies oxygen for reaction at unsaturated carbon atoms of the oil, to effect epoxide addition thereto. In this connection, it should be explained that the water supplied at inlet 5, which may be merely mildly alkaline or may be a solution of a suitable reagent or catalyst, mixes with the oil in the uppermost of the trays 6, and passing with the oil to successively lower trays in the series throughout the height of the reactor, is maintained in a condition of intimate admixture with the oil by the agitation provided by the air streams which are passed therethrough. This water is, as has been explained, necessary to form hydroxyl group additions by hydration at the points of epoxide formation. After passing over successive trays 6, the oil and water are discharged by a final down pipe 26 to region 27 at the base of the reactor 3, where it separates into a lower aqueous body and an upper body of oil. An oil-water interface level regulator 28 of usual construction is provided, and operates in association with pump 4, and pump-flow regulator valve 29, to draw off the aqueous layer from chamber 27 and thus to maintain an approximately constant level of the oil-water interface 30.

The water desirably is in part recycled continuously, part being drawn off by way of connection 31 and a fresh supply being introduced by way of connection 32 under the influence of pump 4. This is of importance, if the water content be associated with a suitable oxygen-supplying reagent, such for example as potassium permanganate or hydrogen peroxide, because it provides for the addition of fresh solution of appropriate concentration without wholly drawing off the solution which has passed through the reactor. If so desired, however, all the used aqueous solution may be withdrawn and fresh solution supplied. As water is drawn off by way of draw-off connection 31, pump 4 maintains the

water volume in reactor 3 constant by supplying a quantity of water equal to that which is drawn off plus any water which may escape as vapor or entrainment by way of vapor outlet 25.

The preferred temperature at which the hydroxylation is effected will depend upon the kind and condition of the oil, and other operating variables, but in general the reacting temperature is as high as may be used without effecting substantial epoxide decomposition and the formation of fixed oxidation products in the oil. As above noted, the preferred temperatures for hydroxylation lie within the approximate range of 130° F. to 250° F. The oil may be subjected to different rates or intensity of reaction as it progresses through the reactor, by maintaining the oil while passing over different pairs of reacting trays, or different individual trays, at determinate different temperatures.

20 The temperature control in the apparatus is obtainable by supplying a temperature regulating fluid to the jacket spaces 9 in each of the reaction trays 6. As shown, these jacket spaces are in communication with a source of heating fluid, such as hot water or steam, as by way of connection 34, and with a source of cooling water as by way of connection 35. The supply of both such temperature controlling media is under the control of a temperature regulating valve 36, having 25 a heat-sensitive element 37 subjected to the influence of the temperature of material flowing over the aerating, or reaction, trays. As shown, the trays are connected in pairs, heating and cooling media being supplied by way of regulating 30 valve 36, to the lower tray of each pair of branch inlet connection 10a and to the jacket space of the tray next above by way of connection 10. Obviously, the temperature regulating means may be modified independently to regulate the temperature in each such tray. Branch outlet connections 11 lead from the upper member of each pair of trays to a common discharge line 11a for heating and cooling fluids.

35 By connection of such sort, heating or cooling fluid is supplied to maintain each region of the reactor 3 at the desired temperature to which the automatic control organization is set, or which it is constructed to maintain. It may here be noted that the epoxidation reaction is strongly 40 exothermic.

45 Pressure within the reactor may, if desired, be controlled by communication with sources of superatmospheric and subatmospheric pressure. In the event water or a water solution of an oxidizing reagent is omitted and steam is supplied by way of steam inlet connection 260 and utilized as the sole hydrating means, the interior of reactor 3 is preferably maintained at a suitable reduced pressure substantially to avoid condensation of 50 the steam. For example, when effecting the hydroxylation reaction to the oil at a temperature of 175° F. with the use of steam, the reactor would preferably be maintained by any suitable means, at a pressure of about 20 inches of mercury. Under other circumstances, superatmospheric pressure may be used, to increase the solubility of oxygen and hydrating medium in the oil.

55 I have discovered that the use of steam tends to render the operation of the hydroxylation reaction more selective with respect to the points of unsaturation in the molecule which are attacked. This is apparent from consideration of the manner in which the oil undergoing treatment is handled in the apparatus. The oil while passing in a 60 sinuous manner over the several reaction trays 70

75

of a typical commercial size apparatus as described is progressively subjected to the influence of and intimately contacted by a very great number of jets of air issuing from the closing spaced slots on the lower edges of the bubble caps. Thus, the effect in the apparatus is repeatedly to mix the oxygen-supplying and hydrating media with the oil stream in the several reaction trays of the apparatus. Such mixture is made, as has been shown, in a manner to effect a high order of intimacy. The air is in the form of bubbles, although the bubbles are very small, and the water, which may hold in solution an additional oxygen-supplying or catalyzing reagent, is mixed intimately with the oil in droplets of small dimension by the action of the air.

The effectiveness of the procedure thus depends upon the repetitive treatment of the oil in the several reaction trays over which it successively passes. Such treatment, which brings a limited proportion of the oil molecules effectively into contact with available oxygen atoms and water molecules in each zone of treatment during the progress of the oil through the reactor, is effective because the oil in relatively small volume is repeatedly subjected to hydroxylating media under hydroxylating conditions. My preferred practice, insofar as this apparatus is concerned, is to conduct the process to effect throughout the body of the oil at least substantially complete hydroxylation of the double bonds at the 12-13 position in the molecules of linoleic acid glyceride and at the 15-16 position in the molecules of linolenic acid glyceride.

It is not difficult to conduct the hydroxylation step in apparatus of this sort in a manner to obtain the result above indicated, because the tendency so to function is inherent. A prime requisite is that the water supply be adequate, with respect to efficiency, fully to hydrate the epoxide addition as it is made. Thus the temperature being within the approximate range of about 130° F. to 250° F., in the presence of an abundance of water, it is possible to hydroxylate the unsaturated carbon atoms of the oil molecules approximately to the maximum extent without substantial formation of permanent oxidation or objectionable ring compounds. If in beginning a run, samples show an undue proportion of fixed oxidation products, the volume of water supplied is increased, and if the condition persists the temperature is reduced to a degree sufficient to avoid such contamination. In the apparatus under consideration, the preferred time of treatment depends upon the rate at which the oil is supplied. This will, of course, vary with specific apparatus designs, individual oil, and the other conditions of the process. A preferred procedure is to test a sample for its order of hydroxylation soon after the beginning of a run and accordingly to adjust the several operating variables.

The oil which has been subjected to the hydroxylating treatment, and which lies as an upper layer on the water in the base of the reactor 3, is continuously withdrawn at an adjusted rate of discharge by means of a pump 38, and an oil level controller 39, operable by way of pump-flow regulating valve 40 to maintain the upper surface of the oil in the base of the reactor at an approximately constant level.

Desirably, drawoff line 41, which leads from the interior of the reactor 3 to the pump 38, is provided with a valved drawoff connection 41a by which test samples readily may be taken off from time to time.

Oil drawn off by pump 38 is delivered to apparatus for conducting the second, or dehydrating, step of the process by way of supply line 42. Desirably, supply line 42 passes by way of an oil heater 43 and de-aerator 44, in order to remove from the oil any entrained or dissolved air, loosely-bound oxygen, or moisture, which would cause excessive foaming and promote the formation of undesired compounds in the dehydroxylation treatment. Thus, oil passing by way of supply line 42 is first heated, as in the heater 43, and is then delivered to de-aerating vessel 44, which is maintained under suitably reduced pressure, by which entrained or dissolved air and moisture are removed in the form of vapor by way of vapor outlet connection 45. The reach of the discharge line 42 leading from de-aerator 44 is provided with a pump 46 leading by way of connection 47, to a heat-exchanging element 48 in condensive dehydroxylation reactor 50. From heat-exchanging structure 48, supply line 49 leads through other preparatory apparatus elements to inlet 51 adjacent the top of the reactor.

The preparatory apparatus elements, as shown, comprise a catalyst-mixing chamber 52, in which the oil is intimately mixed with suitable condensive dehydration and hydrolysis-promoting catalysts from a supply tank 53, and proportioning catalyst-feed device 54 of common construction. As shown, catalyst supply tank 53 is provided with agitating means 53a by which the catalyst may be mixed with a small portion of oil, which desirably is identical with the main body of oil subjected to treatment. Between catalyst mixer 52 and inlet connection 51, supply line 49 leads through an oil heater 55 in which the flowing stream of oil is brought initially to a temperature which at least approximates that of the condensive dehydration reaction to which it is to be subjected.

Condensive dehydroxylation reactor 50 desirably is constructed throughout of a metal capable of resisting the corrosive action of the materials introduced into it or produced in conducting the process. Its shell is a cylindrical columnar body of adequate cross-sectional area to provide for the several effects to be created in it, and is of a height adequate to provide a relatively great length of travel of oil passed downwardly through it and subjected to the condensation reaction in its passage. Within reactor 50 and of a length approximating the height of the reactor shell, there is a tubular element divided vertically into an upper heated reaction section 56, and a lower cooling section 57, which forms part of the heat-exchanger 48, by which the incoming oil is heated and by which the temperature of oil treated in the reactor is rapidly lowered.

Pre-heated oil entering reactor 50 by way of inlet connection 51, is first received by a separating-vaporizer 58, in which any fatty acids, or other volatiles which may be carried by the heated oil flash-vaporize under the pressure conditions existing interiorly of the reactor, and pass by way of vapor outlet 59 to suitable condensing and collecting means not shown. It may be explained that the interior of reactor 50 surrounding the tubular structure 56 and 57, desirably is maintained at a reduced pressure, for example under a pressure of 3 to 5 mm. of mercury, by suitable vacuum-creating means, not shown. The oil in substantially liquid form passes from vaporizer 58 by way of a connection 60, to an oil distributor 61 at the top of reactor tube 56, from which it is passed outwardly by way of a number of narrow,

closely spaced slots 62, and is uniformly distributed on the outer surface of tubular reaction element 56 down which it flows by gravity in the form of a relatively thin layer or film, which may be about .065" and even less in thickness. The oil film travels downwardly over reactor tube 56 rapidly under gravity, as for example, at a speed of 10 to 15 lineal feet per second, the speed at which the oil in such film travels depending somewhat upon the viscosity of the oil and the effect of vapor formed by the reactions which take place in the oil film.

Any suitable agency such as hot vapors, hot circulating fluids, or electricity for heating reactor tube 56 to the relatively high temperature required for the "flash" condensive reaction may be used, preferred heating means being shown in Fig. Ib and in Figs. IV and V of the drawings. As shown therein, reactor tube 56 is electrically heated by means of electric current which is supplied by way of transformer 63 and electrical connections 64, 64a. Transformer 63 receives current from a line 65 leading to any suitable current source, by way of automatic control switch 66, operable under the influence of a thermostatic regulator 67 and which has electrical connections 68 to transformer 63 and connection 69 with a thermocouple 70, which last-named element extends through the reactor shell into operative relation with the heated surface of reactor tube 56.

Electrical connection 74 between low-resistance tube 71 and high-resistance tube 75, together with its insulator, is engaged in a liquid-tight partition 76 arranged at the junction between heated reactor tube 56 and lower cooling tube 57.

The film of oil, passing rapidly down the surface of reaction tube 56 is raised quickly to a relatively high reaction temperature lying within the approximate range of 500° F. to 700° F., such as a temperature of about 550° F.; and continuing downwardly over the surface of cooling tube 57, still in the form of a thin, rapidly flowing stream, is cooled quickly to a temperature below that which would produce in it substantial heat polymerization. For example, it is rapidly cooled to a temperature of about 275° F., or lower, by heat exchange with the cooler stream of oil flowing upwardly in annular space 87 in direct contact with the inner surface of cooling tube 57. The treated oil thus cooled collects in space 89 at the base of the dehydroxylation reactor, and is continuously delivered from it by way of a discharge connection 90 for further treatment, or for storage.

I have found that there is a substantial difference in the temperature at which the hydroxyl groups in different positions in the carbon chain react or condense with adjacent hydrogen atoms, the hydroxyl groups at the remote carbon position reacting at a substantially lower temperature than those groups nearer the glycerol group in the oil molecule. This difference in reaction temperature is quite substantial, and may amount to as much as 50° F. or more. While "flash" dehydration is desired, if the condensive reaction should take place instantaneously throughout all regions of each of the hydroxylated oil molecules, upon contact in the upper region of the reactor tube, the immediate evolution of substantial amounts of water produced by the condensive reaction would result in violent ebullition and oil might thus be thrown

mechanically from the surface of the reaction tube.

In my condensive dehydroxylation step, the condensation reaction is in effect a flash reaction, inasmuch as it usually takes place within a period of a few seconds, at a temperature of from about 500° F. to 700° F., rather than in a period in the order of three to four hours at temperatures from about 450° F. to 540° F., when condensive dehydroxylation is conducted in accordance with a batch procedure. That is, in the progress of a thin film of the oil downwardly on the surface of a reactor, such as the surface of the reactor tube 56 of the dehydroxylation apparatus shown, the oil is subjected to condensive reaction temperatures so high that dehydroxylation is substantially complete before it is cooled, as by passing over the cooling surface, such as is provided by the cooling tube 57 of the apparatus shown. As indicated above, it is desirable, however, that the condensive flash reaction should not be so wholly instantaneous as to produce violent mechanical effects in the film of oil subjected to treatment. Thus, I prefer to supply oil which has been pre-heated, as by its use in heat-exchange and subsequent heating in an oil heater, to a temperature which is at least 50° below the maximum temperature to which it is to be brought in the reactor. For example, I prefer to supply the oil at a temperature no higher than from about 450° F. to 500° F., and to bring it during its brief period of contact with the reactor tube to its maximum, or flash, reaction temperature of at least 500° F., so that the zone of the condensive reaction comprises substantially the entire length of reaction tube 56.

By the term "flash" condensive dehydration, I mean a condensive dehydroxylation reaction in which the oil is subjected for a very short period not substantially exceeding 1 minute to elevated temperature from about 500° F. upward and below a temperature at which heat-decomposition of the oil will take place during the period of the treatment. I have found that such "flash" dehydration should be performed upon an attenuate body of the hydroxylated oil, such as the thin, circular stream, or film, of oil which the condensive dehydroxylator above described is organized to present.

The rapid cooling should in each instance bring the oil to a temperature below that at which the viscosity of the specific dehydrated oil is substantially increased by heat reaction.

By operating under subatmospheric pressure, as by maintaining a pressure of 5 mm. of mercury or less within the reactor, the flowing stream, or film, of reacting oil is maintained in substantially anhydrous condition by the continuous removal of water produced by the condensive reaction substantially as it is formed. The prompt removal of the water evolved by the condensive reaction from the flowing film of oil and the use of relatively high reacting temperature, provide conditions under which the rate and the extent of the dehydrating reaction may approach the maximum. Water being an end product of the reaction, tends strongly to inhibit its progress. Instantaneous removal of water, and the presentation of the oil in a thin stream, or film, greatly accelerates the condensive reaction at the temperatures to which the oil is subjected. Because of the very brief period of time during which the oil is subjected to high temperature in effecting the condensation reaction, such high temperature may be utilized without

injuring the oil as it would were the oil subjected to it for an extended period of time.

I have also found that under the above recited reacting conditions, and particularly at the higher temperatures within the given range, the use of condensive dehydrating-promoting catalysts is not important, and that in the treatment of many oils the condensive dehydroxylation may be completed to an adequate degree in the substantial absence of such catalysts.

It may be stated that my flash dehydrating effects approximately complete dehydroxylation with the production of an oil having the desired high order of conjugate unsaturation, without involving as an incident to such reaction heat-polymerization of the oil, which the further treatment to which the oil is subjected or the use to which the oil is to be put might render objectionable.

An exemplary form of hydroxylation reactor purposed particularly for highly selective hydroxylation of the oil, is shown in Fig. VII of the drawings. This reactor, the shell of which is designated by reference numeral 95, receives oil for treatment through line 96 under the influence of feed pump 97, and by way of flow indicator 98, and oil heater 99. Oxygen-supplying gas, for example air, is supplied in suitable quantity and under suitable pressure by means of air blower 100, flow indicator 101, air heater 102, and by way of line 103, to the interior of reactor shell 95. Steam, or hot water, is supplied by way of connection 104, and flow indicator 105, to air-steam mixer 106 in suitable quantity to effect hydroxylation of the epoxide addition formed by reaction between unsaturate carbon atoms in the oil and oxygen supplied by the air. Both oil supply line 96 and air-steam supply line 103 connect with an atomizer 107, by which the oil is discharged into the interior of the reactor in the form of a fine mist, or spray, intimately commingled with the oxygen-supplying gas, and with the hydrating medium, such as steam or water vapor. By thus effecting highly intimate and immediate contact between the oil and the oxidizing and hydrating media, there is a substantially instantaneous reaction, or sequence of reactions, by which hydroxylation of highly selective sort is effected.

Desirably, the mixture of air and steam is supplied to atomizing device 107 at a suitable hydroxylation temperature within the range above noted, such as a temperature of 175° F., and desirably, the oil for treatment is supplied to the atomizer at a similar temperature. For this purpose, oil heater 99 is provided with a heating medium, such as steam, by way of a connection 99a, supplied under the control of a temperature regulator 99b. Similarly, air heater 102 desirably is supplied with pre-heating steam by way of a connection 102a, under the control of a temperature regulator 102b. Assuming, for example, that oil is supplied to the reactor at a rate of 1000 lbs. per hour, I have found an air supply of 225 cubic feet per minute adequate to effect epoxide addition to selected unsaturated carbon atoms in the oil molecule without substantial formation of fixed oxidation compounds therein, providing that the steam, or other source of hydrating water at a desirably high temperature, is also supplied in a quantity sufficient instantaneously to hydrate and thus to make hydroxyl addition to the unsaturate carbon atoms as epoxide formation is effected. If it is desired

to accelerate epoxide formation, and consequently to accelerate hydroxylation, a minute amount of any suitable oxidation-promoting catalyst, such for example as a compound of cobalt or the like, preferably in oil soluble form, may be supplied with the oil. Preferably the reaction chamber is maintained at a suitably reduced pressure, such as a pressure of from 20 to 25 in. of mercury, in order to prevent condensation of the hydrating steam. Reduced pressure has another advantage in that because of expansion the volume of the air is greater than at atmospheric pressure, thus providing greater contact efficiency between the oxidizing air and hydrating steam and the minutely divided oil particles in the form of mist produced by the atomizer.

Briefly to consider the organization of the hydroxylation reactor, an inner shell 108, concentric with the outer shell 95, desirably is supported within the reactor shell by means of spiders 109, to provide an annular space 110, for the escape of unreacted air and other vapors from the reactor by way of vapor outlet 111. An oil level control device 112 is connected in the lower region of the reactor, and is operable by way of an oil discharge pump 113, and flow regulating valve 114, to maintain the oil within the reactor at a substantially constant level. Because epoxide formation is a reaction which is highly exothermic, cooling coil 115 desirably is provided to establish heat-absorbing conditions in the interior of the reactor.

In operation, the fine oil particles under the influence of gravity and because of the velocity imparted to them by atomizer 107, fall to the lower part of the reactor. There the hydroxylated oil is retained for a sufficient period of time under the influence of oil level control device 112 to effect gravity separation between the oil and any water which may be mixed with it. The oil from the oil stratum 116 is constantly removed by means of pump 113, and passes by way of discharge line 112a to the dehydrogenating reactor. Separated water is drawn off by valved connection 117 to maintain an approximately constant level of the oil-water interface.

Excess and oxygen-depleted air, together with steam and any other vaporous products of the reaction, escape by way of annular space 110 to vapor outlet 111, passing on their way through oil entrainment separating louvres 118 which act substantially to remove entrained oil particles from the discharged vapors. It is to be understood that oil passing by way of line 112a to the condensive dehydrogenation reactor 50 as with the form of hydroxylating apparatus previously discussed, desirably passes through a similar oil heater and de-aerator to remove any entrained or dissolved air, loosely-bound oxygen, or moisture from the oil; and that the heating and other steps preparatory to delivery of the oil to the dehydrogenation reactor are similarly conducted.

I have found when using the above described form of flash hydroxylation reactor, because of better contact efficiency between the oil and the oxidizing and hydrating media, the brief or practically instantaneous time of the exposure of the oil to the treatment, and the more exact regulation of the variables controlling the reaction, that substantially greater reacting temperatures may be utilized in the treatment without substantial formation of fixed oxidation and other objectionable ring compounds in the oil, than when treating the oil by other methods involving relatively longer times of treatment

which offer greater opportunity for the formation of such objectionable compounds, thus not only increasing the rate of production many times, but also producing a more uniformly treated product. The flash hydroxylation may be utilized to effect a mild and but partial hydroxylation to the oil by selective diminution of the operating variables such as air, temperature, and oxidation catalyst, or to effect a more intense hydroxylation of the oil by selective intensification of those variables.

I shall now give specific exemplification of runs which have been conducted in accordance with the procedure of my method and in apparatus as herein shown and described. It is to be understood that such exemplification is in nowise restrictive, but that it will be subject to wide variation in response to a number of conditions. Even different batches of the same sort of oil preferentially ask accommodation in the conditions of their treatment, and minor variations in the structure of the apparatus also cause variations in the conditions most to be preferred. The example given immediately below is to be understood as conducted on linseed oil as the starting material, such oil being of a commercial quality which has been subjected to the usual refining treatment for the removal of gum, mucilage, and other colloidal and suspended impurities, and for the removal of excess free fatty acids.

The example is to be considered as illustrating a treatment in the hydroxylation apparatus shown in Fig. Ia of the drawings, and in the dehydroxylation apparatus shown in Fig. Ib of the drawings, or in closely analogous apparatus. It will be noted that in the example all of the hydrating water is supplied in the form of steam. This is my preferred procedure for several reasons. In utilizing steam, the hydrating medium being in the form of vapor, may be initially commingled with the air which supplies oxygen for epoxidation, and being in the form of vapor is more uniformly and intimately commingled with the air than is possible when utilizing water in liquid state. Thus, in the use of steam, a water molecule for hydration is associated so directly with an oxygen molecule of the air that the conditions favor simultaneous contact of both with the oil molecule, to cause instantaneous hydration of the epoxide as it is formed. Such mechanism serves to inhibit the formation of permanent oxidation products, and renders hydroxylation of the oil molecules more selective. Additionally, the use of steam avoids the tendency toward emulsification which is present when water in liquid state is used as the hydrating medium.

*Example 1*

In accordance with this procedure, linseed oil for treatment was supplied to the hydroxylating reactor of Fig. Ia in the manner described in the description of that apparatus, at a reacting temperature of about 165° F., and at the rate of about 1000 lbs. per hour. Air for oxidation, pre-heated to a temperature of about 165° F., was supplied at a rate of about 275 cubic feet per minute. Steam for hydration was supplied at a rate of about 225 lbs. per hour, being in accordance with the disclosure of the reactor to which reference is made, commingled with the air to pass upwardly with it through the several reaction trays of the apparatus. A reduced pressure of about 20 inches of mercury was maintained within the reactor during the

process, substantially to prevent condensation of the steam at the reaction temperature. The oil subjected to treatment passed downwardly through the reactor in the manner described in connection with the apparatus; and with the size and arrangement of apparatus used, the oil was subjected to treatment for a period of about 30 minutes during its progress through the reactor.

Treatment under the conditions given resulted in the selective addition of hydroxyl groups to the remote pairs of unsaturate carbon atoms of the linolenic and linoleic acid glycerides of the oil composition without substantial oxidation, or hydroxyl group addition, to those unsaturate carbon atoms of the linolenic, linoleic, or oleic acid glycerides lying next toward the glycerol radical of the glycerides. In terms of hydroxyl value, the treated oil showed a hydroxyl value of about 210 as compared with an initial hydroxyl value of about 4.

The linseed oil hydroxylated as above, in preparation for treatment in a dehydroxylator of the sort shown in Fig. Ib, was subjected to a de-aerating temperature and reduced pressure of about 3 to 5 mm. of mercury, and was raised from a temperature of about 180° F. to about 360° F. with addition of a suitable dehydrating catalyst, which specifically consisted of about 0.5% sodium acid sulphate. The oil was then heated to a temperature of about 475° F. and free fatty acids and other volatile compounds were flashed off.

The oil thus prepared for condensive dehydroxylation was then treated in accordance with the procedure given in the description of the apparatus of Fig. Ib. As closely as could be estimated, the oil was brought in a thin film and under a reduced pressure of about 3 to 5 mm. of mercury to a temperature progressively increased during a period of about 5 seconds to a maximum of about 610° F., and was immediately cooled to a temperature of about 300° F. As will have been apparent from the discussion associated with the description of the condensive dehydroxylating apparatus, this "flash" condensive dehydrating primarily is rendered possible by the fact that the oil is subjected to treatment in a thin film, so that within a short period of time it may be raised to a high temperature and the temperature reduced to below a point in which heat-polymerization will occur in the oil.

During the treatment the dehydroxylating reactor was maintained under a reduced pressure of about 3 to 5 mm. of mercury, and the water evolved by the condensive reaction was instantaneously removed from the thin rapidly flowing stream of oil. Likewise relatively volatile materials in the oil, such as fatty acids, reduced glycerides, and other volatile non-drying contaminates, such as aldehydes, ketones, and oil decomposition compounds which may have resulted from the prior treatment to the oil were vaporized and eliminated from the flowing stream of the oil. The treated oil was thus substantially free of hydroxyl and other addition groups, and of saturated and other non-drying contaminates.

The oil subjected to the foregoing treatment had been converted from an oil having the usual drying properties of linseed oil to one having a high degree of conjugate unsaturation, with high heat-reactivity and improved film-forming properties. The oil had been converted from one initially requiring about 175 minutes to gel under standard gelation test conditions, to one that will 75 gel under the same conditions in about 15 min-

utes. The oil also had a desirably low viscosity, its increase in viscosity by the above described treatment being from an initial of about 4 poises to about 10 poises, and because of the minimized formation of fixed oxidation products during the hydroxylating reaction the oil had a desirable light color. Because of the distilling or stripping action at high temperature and reduced pressure, the oil was substantially neutral, having a F. F. A. of about 0.15%.

### Example 2

A mixed oil, consisting 50% of commercial refined linseed oil as in Example 1 and 50% of refined desaturated soya bean oil, was subjected to treatment in apparatus combining a hydroxylator as in Fig. Ia with a condensive dehydroxylator as in Fig. Ib. The conditions were substantially identical with those given above in Example 1. By this treatment, the mixed oil was converted from one requiring about 60 minutes to gel under standard gelation test conditions, to one that gelled under the same conditions in about 10 to 12 minutes. The viscosity of the treated oil was about 10 poises.

It may be noted that in treating soya bean oil and like oils having a large proportional content of saturates and semi-saturates it is desirable, as hereinafter more fully explained, to desaturate the oil before treatment.

### Example 3

A soya bean oil which had been refined, as was the linseed oil of Example 1, but which contained its total initial content of the glycerides of saturate fatty acids and oleic acid glyceride, was subjected to treatment in a hydroxylatation reactor such as is shown in Fig. Ia and a condensive dehydroxylator such as is shown in Fig. Ib. In treating this oil, hydroxylatation was carried to a point of substantial completion rather than selectively performed as in the treatment of the linseed oil and the mixed oil of Examples 1 and 2. In so doing, the conditions of the hydroxylatation reaction were intensified. Assuming that the oil was fed to the reactor at a rate of about 1000 lbs. per hour, air heated to about 190° F. was supplied at a rate of about 325 cubic feet per minute. Hydrating steam was supplied at a rate of about 350 lbs. per hour in order to give assurance of an abundance of hydrating medium. The oil itself was pre-heated to the same temperature as the air, namely to about 190° F., in order to provide a reaction temperature in that order. The reactor was maintained at a reduced pressure of about 15 inches of mercury in order to prevent condensation of the steam.

The untreated soya bean oil required about 220 minutes to gel under standard gelation test conditions, and the treated oil gelled under the same conditions in about 22 minutes.

#### Example 4

Linseed oil of the sort and in the condition described was subjected to hydroxylation in a hydroxylation reactor of the sort shown in Fig. VII of the drawings, the treatment as in Example 1 being purposed to give after condensive dehydrogenation an oil in which only the remote unsaturate carbon atoms in the carbon chain of the glycerides attacked were affected. In this treatment the linseed oil was supplied the reactor at a rate of about 1000 lbs. per hour, the oil being pre-heated to a temperature of about 175° F. to 185° F. Air heated to the same temperature was supplied at a rate of about 225 cubic feet per

minute and was atomized with steam supplied at a rate of about 400 lbs. per hour. The interior of the reactor was maintained at a reduced pressure of about 20 inches of mercury.

5 The oil treated by this procedure corresponded very closely to the oil treated by the procedure of Example 1.

It is to be understood that in all of Examples 2, 3 and 4, the condensive dehydroxylation operation and the steps by which the hydroxylated oil was prepared for that stage of the process were identical with those described in Example 1.

The foregoing examples point the direction in which adjustment may be made in the several variables involved in the process, in accordance with the properties of the starting oil, the desired properties of the product oil, and the influence of the apparatus used upon preferential procedure.

20 Returning to the chemical mechanism involved in my novel treatment of drying oil, it will be considered that linolenic acid glyceride and linoleic acid glyceride are the principal glycerides acted upon in the treatment. It will  
25 be assumed, also, that the treatment has been a selective one in which hydroxylation followed by condensive dehydroxylation has been effected at a desired point of attack in the acid radical of the oil molecule. The following formulae will  
30 illustrate the change effected in the acid radical of the glyceride, the glycerol radical being omitted for the sake of simplicity.

The linolenic acid radical ( $H_30C_{18}O_2$ ) may be represented as follows:

### Formula A



Observing the formula, it is seen that the carbon atoms in the 9-10 positions are linked with a double bond, as are also the carbon atoms in the 12-13 positions and in the 15-16 positions.

If, then, hydroxyl addition is made at both the carbon atoms in the 15-16 positions we obtain Formula B, as follows:

### Formula B ( $\text{H}_{32}\text{C}_{18}\text{O}_4$ )



Formula B shows the selectively hydroxylated acid radical before condensive dehydroxylation, with both the carbon atoms in the 15-16 positions saturated by addition of an OH group.

Formula C shows the acid radical after condensive dehydroxylation as follows:

### Formula C<sub>18</sub>H<sub>28</sub>O<sub>2</sub>



In this modification of the structure, a hydrogen atom in the 14 carbon position and a hydrogen atom in the 17 carbon position have been involved in a condensative reaction with adjacent hydroxyl groups by which two molecules of water are formed. The removal of those hydrogen atoms has resulted in the formation of double bonds between the 16 position carbon and the 17 position carbon, and between the 14 and the 15 position carbons. The double bond linking the carbons in the 13 and the 12 positions has re-

21

mained unaltered, as has also the isolated double bond between the carbons in the 9-10 positions.

From the above, it will be seen that the result is to produce a novel glyceride, in which the acid radical has three double bonds in conjugate relation, in addition to one initial double bond which is still in non-conjugate position. Also, it will be seen that at each original pair of unsaturate carbon atoms the hydrogen atoms adjacent both the carbons have gone to form the two molecules of water, so that double bonds have been introduced in both directions from the double bond originally present. 5 10

The effect is analogous in the case of linoleic acid glycerides. The formula for linoleic acid is as follows:

*Formula D* ( $\text{H}_{32}\text{C}_{18}\text{O}_2$ )



It will be seen in this formula that the linoleic acid radical has two isolated double bonds, one between the carbons in the 9-10 position and the other between the carbons in the 12-13 position. It has been explained that hydroxylation is effected at the 12-13 carbons more readily than at the carbons in the 9-10 position. The linoleic acid glyceride being selectively hydroxylated, the structure will then appear as follows:

### Formula E ( $\text{H}_{34}\text{C}_{18}\text{O}_4$ )



This effect is to add hydroxyl groups at the carbon atoms in the 12 and 13 positions, which upon condensive dehydroxylation, as shown above, involves the hydrogen atoms in the 11 and 14 carbon positions, the modified structure derived from the linoleic acid radical of the oil molecule then will have double bonds in the 9-10, 11-12, and 13-14 positions in accordance with the following formula:

### Formula F ( $\text{H}_{30}\text{C}_{18}\text{O}_2$ )



This increase in unsaturation by formation of the three conjugated double bonds is in this instance caused by the saturation and subsequent elimination of the original double bond in the 12-13 position and the formation by dehydration of double bonds at the 11-12 and 13-14 carbon positions. It will be noticed that the introduced unsaturation gives three double bonds in conjugate relation.

For the purpose of comparison, the formula for eleostearic acid is here given as follows:

### Formula G ( $\text{H}_{30}\text{C}_{18}\text{O}_2$ )



If we assume that the oil treated is linseed oil, consisting 24% of linolenic acid glyceride, and 62% linoleic acid glyceride, with 5% oleic acid glyceride, and 9% of the glycerides of saturated fatty acids, it will be seen that the treated oil has a total reactivity corresponding very closely to that of China-wood oil, although the points

of unsaturation are, as shown, slightly different from those of eleostearic acid glyceride.

If, however, my treatment be conducted on a starting material which is an oil such as soya bean oil composed about 6% of linolenic acid glyceride, 50% of linoleic acid glyceride, 30% oleic acid glyceride, and about 14% of the glycerides of saturated fatty acids, there is a different emphasis on the subsequent treatment of the dehydroxylation product. If soya bean oil, for example, be moderately hydroxylated (i. e. if hydroxylation be restricted to the remote unsaturate carbon atoms in the carbon chains of the molecules attacked) and then subjected to condensive dehydroxylation, the resultant product derived from natural soya bean oil would consist about 50% of a glyceride responding substantially to the formula for eleostearic acid glyceride, about 6% of a glyceride containing three conjugate double bonds, and one non-conjugate double bond, about 30% of oleic acid glyceride, and may have about 14% of unchanged glycerides of saturated fatty acids. Such product oil is a good drying oil. Further to improve the properties of such product oil, the content of the glycerides of saturated fatty acids and of unchanged oleic acid glycerides desirably may be removed by solvent extraction, in accordance with any of the various solvents and procedures which are well-known for the separation of saturates and semi-saturates from the unsaturate fatty acid glycerides; and with any of the well-known suitable solvents for that purpose, such as those of the class comprising acetone, ketones, and the higher molecular weight alcohols. It is to be understood that linseed oil and other oils treated in accordance with my method similarly may be subjected to solvent extraction, in the event their non-reactive content is too great to give them the ability to form films of a desired hardness. It is also to be understood that such oils may be subjected to solvent extraction substantially to remove the saturated non-drying components from the oil prior to subjecting it to treatment and the concentrated unsaturated components utilized as the starting material for my product oil.

my product oil.

An instance in which selectivity is of particularly great importance is presented by the fish oils, which contain in addition to a moderate content of linoleic acid glyceride and linolenic acid glyceride, a moderate content of the highly unsaturated and non-conjugate glycerides, such as clupanadonic acid, containing more than 18 and up to 26 carbon atoms in their carbon chain, and initially having from 4 to 6 points of unsaturation in their structure.

I have found in treating such oils to obtain what is in practical effect a "flash" hydroxylation, as in the manner which I have described with reference to a reactor of the type shown in Fig. VII of the drawings, that in the hydroxylation treatment the addition of hydroxyl groups to the linoleic acid and linolenic acid radicals proceeds proportionally with the addition of hydroxyl groups in the fish oil acid radicals. The increased unsaturation and conjugation in those radicals is balanced sufficiently by the greater length of the carbon chain and the proportionally greater molecular weight as compared with linoleic and linolenic acids, to give an oil of approximately uniform hydroxylation.

It may be stated that my invention resides primarily in treating a drying oil having a substantial content of those unsaturated fatty acid radi-

23  
cals which contain at least 18 carbon atoms, and which have at least two points of unsaturation, by hydroxylation followed by condensive dehydroxylation, to produce an oil having, by virtue of increased unsaturation and introduced conjugation, increased heat-reactivity. Also, my invention resides in so controlling or apportioning the hydroxylation stage of such treatment that in the oil the acid radicals of the above noted sort to which the treatment is directed are hydroxylated either fully or in less than maximum order, with consequent control of the extent to which their polymerizing reactivity is increased; and resides in condensively dehydroxylating by means of a "flash" dehydration which effectively dehydroxylates the hydroxylated oil, without decomposing the oil or unduly increasing its viscosity.

To the extent that the starting oil consists of "reactive" glycerides, that is glycerides of fatty acids having at least 18 carbon atoms in the carbon chain and at least two pairs of carbon atoms linked by double bonds, the oil is increased in iodine value from a very substantial percentage increase to an increase of more than 100%. The increase in unsaturation, or iodine value, is inevitably accompanied by conjugation, because each double bond which originally links two carbon atoms is replaced by two double bonds each linking one of the originally unsaturated carbon atoms with another adjacent carbon atom.

Considering the two commercial drying oils considered above, namely linseed oil and soya bean oil, it has been explained that the linseed oil has an initial iodine value of about 180 and the soya bean oil has an iodine value of about 140. By selectively subjecting these oils to treatment in accordance with my method under controlled conditions, I am able to increase the iodine value of the linseed (with conjugation) to from about 200 to about 360. Similarly, I am able to increase the iodine value of the soya bean oil (with conjugation) to from about 150 to about 250.

By virtue of an hydroxylation treatment which is effective rapidly to produce epoxide formation with substantially simultaneous hydration, the oil is approximately free of permanent oxidation and other objectionable compounds. By virtue of condensive dehydration effectively performed the initial viscosity of the product oil is not undesirably increased.

My drying oil product thus is an improved oil resultant from an oil having a substantial initial content of non-conjugate unsaturated reactives, in which unsaturation has been increased with an increase in conjugation which matches the increase in unsaturation. That is, increased unsaturation is effective proportionally to product conjugation. The position of the unsaturation and of the conjugation in the molecules of the treated oil is determinate.

The foregoing disclosure of my invention has been made full and detailed, in order that the invention may be fully understood and that full benefit may be derived from it. As above indicated, however, it is to be taken that such detail disclosure is descriptive and not restrictive, and that the scope of my invention is to be limited only by the definition of my invention as contained in the appended claims.

I claim as my invention:

1. The method of improving the heat reactivity and film forming properties of non-conjugate glyceride oils containing a substantial proportion

of components having two or more pairs of unsaturated atoms in their carbon chain, which comprises subjecting, a confined continuously flowing stream of the oil divided into a plurality of successive shallow pools while passing downwardly through a treating vessel, to selective hydroxylation by intensively blowing said pools in the presence of a hydroxylating catalyst with an upwardly flowing stream of oxygen containing gas, intimately mixed with hydrating steam in amount sufficiently greater than the theoretical amount required to hydrate the epoxy groups to insure the hydration of all of the epoxy groups selectively added thereto by said blowing at a selective epoxidation reaction temperature within the range of 130° F. to 250° F. for approximately 30 minutes, sufficient to selectively add hydroxyl groups to the remote pairs of unsaturated carbon atoms of said unsaturated components without substantial oxydative polymerization thereof or oxygenation of the 9-10 unsaturated carbon atoms present in said oil composition, then quickly removing such hydroxylated oil from the zone of oxidation, removing free water and air therefrom and subjecting the oil to flash-dehydroxylation by quickly heating a thin rapidly flowing stream at a reduced pressure in the presence of a dehydrating catalyst at a determinate flash dehydrating temperature within the range of 500° F. to 700° F. for a brief, substantially non-thermal polymerizing period of time about one minute or less correlated to said dehydrating temperature, effective to produce a substantially non-oxidized, non-polymerized conjugate type drying oil product containing a substantial proportion of glycerides having one more double bond than the corresponding unsaturated components of the said starting oil from which they were derived.

2. The method as set forth in claim 1 wherein said glyceride oils include linolenic glyceride and said epoxidation temperature is within the range of 130° F. to 190° F. and wherein hydroxyl groups are selectively added at the 15-16 carbon positions of said linolenic glyceride, to produce an oil product having a substantial proportion of glycerides having double bonds at its 9-10, 12-13, 14-15 and 16-17 carbon positions.

3. The method as set forth in claim 1 wherein said glyceride oils include linoleic glyceride and said epoxidation temperature is within the range of 200° F. to 250° F. and wherein hydroxyl groups are selectively added at the 12-13 carbon positions of said linoleic glyceride to produce an oil product having a substantial proportion of glycerides having double bonds at its 9-10, 11-12, 13-14 carbon positions.

4. The method of improving the drying properties of linseed oil as set forth in claim 2.

5. The method of improving the drying properties of soy bean oil as set forth in claim 3.

ROBERT A. CARLETON.

#### REFERENCES CITED

The following references are of record in the file of this patent:

#### UNITED STATES PATENTS

| Number    | Name     | Date          |
|-----------|----------|---------------|
| 1,565,249 | Berry    | Dec. 15, 1925 |
| 2,083,220 | DeGroote | June 8, 1937  |
| 2,194,250 | Turek    | Mar. 19, 1940 |
| 2,278,425 | Colbeth  | Apr. 7, 1942  |
| 2,308,152 | Boone    | Jan. 12, 1943 |
| 2,317,362 | Colbeth  | Apr. 27, 1943 |
| 2,361,793 | Porter   | Oct. 31, 1944 |